



US010392581B2

(12) **United States Patent**  
**Han et al.**

(10) **Patent No.:** **US 10,392,581 B2**  
(45) **Date of Patent:** **Aug. 27, 2019**

(54) **CARBON MATERIAL WICK FOR CANDLE AND CANDLE INCLUDING THE SAME**

(71) Applicant: **Samyoung Machinery Co., Ltd.**,  
Gongju-Si (KR)

(72) Inventors: **Kuk Hyun Han**, Daejeon (KR); **Yea Won Shim**, Daejeon (KR); **Dal Ho Kim**, Daejeon (KR); **Kyung Hwa Ji**, Daejeon (KR)

(73) Assignee: **Samyoung Machinery Co., Ltd.**,  
Gongju-si (KR)

(\*) Notice: Subject to any disclaimer, the term of this patent is extended or adjusted under 35 U.S.C. 154(b) by 12 days.

(21) Appl. No.: **15/649,333**

(22) Filed: **Jul. 13, 2017**

(65) **Prior Publication Data**

US 2018/0023034 A1 Jan. 25, 2018

(30) **Foreign Application Priority Data**

Jul. 22, 2016 (KR) ..... 10-2016-0093056

(51) **Int. Cl.**  
**CIIC 5/00** (2006.01)

(52) **U.S. Cl.**  
CPC ..... **CIIC 5/006** (2013.01); **CIIC 5/004** (2013.01)

(58) **Field of Classification Search**  
CPC combination set(s) only.  
See application file for complete search history.

(56)

**References Cited**

**U.S. PATENT DOCUMENTS**

|                   |        |                |            |
|-------------------|--------|----------------|------------|
| 3,462,235 A *     | 8/1969 | Summers .....  | C11C 5/006 |
|                   |        |                | 431/289    |
| 2004/0137392 A1 * | 7/2004 | Garnys .....   | C11C 5/002 |
|                   |        |                | 431/126    |
| 2009/0042153 A1 * | 2/2009 | Ronen .....    | C10L 1/02  |
|                   |        |                | 431/126    |
| 2012/0148966 A1   | 6/2012 | Ramaker et al. |            |

**FOREIGN PATENT DOCUMENTS**

|                    |         |
|--------------------|---------|
| JP H0841487 A      | 2/1996  |
| KR 200179220 Y1    | 4/2000  |
| KR 100783490 B1    | 12/2007 |
| KR 1020130073481 A | 7/2013  |
| KR 101370867 B1    | 3/2014  |
| KR 101392227 B1    | 5/2014  |
| KR 1020140081875 A | 7/2014  |
| KR 101492333 B1    | 2/2015  |
| KR 1020160000112 A | 1/2016  |

\* cited by examiner

*Primary Examiner* — Ellen M McAvoy

*Assistant Examiner* — Chantel L Graham

(74) *Attorney, Agent, or Firm* — McCoy Russell LLP

(57) **ABSTRACT**

Provided is a wick for a candle including a carbon material. In addition, provided is a candle including the wick for a candle. By using the wick for a candle according to the present invention, it is possible to provide the candle in which a length of the wick combusted at the time of combustion is not long and ash of the wick does not fall.

**12 Claims, 9 Drawing Sheets**



FIG. 1



FIG. 2



FIG. 3



FIG. 4



FIG. 5



FIG. 6



FIG. 7



FIG. 8



FIG. 9



FIG. 10



FIG. 11



FIG. 12



FIG. 13



**FIG. 14**



**FIG. 15**



**FIG. 16**



## 1

CARBON MATERIAL WICK FOR CANDLE  
AND CANDLE INCLUDING THE SAMECROSS-REFERENCE TO RELATED  
APPLICATIONS

This application claims priority under 35 U.S.C. § 119 to Korean Patent Application No. 10-2016-0093056, filed on Jul. 22, 2016, in the Korean Intellectual Property Office, the disclosure of which is incorporated herein by reference in its entirety for all purposes.

## TECHNICAL FIELD

The following disclosure relates to a wick for a candle including a carbon material, and a candle including the same.

## BACKGROUND

A candle may provide a warm and special mood as a natural light source unlike an artificial light source such as electric lighting, and have additional advantages such as deodorization, fragrance, etc., such that use of the candle has gradually increased. The candle is lighting fuel produced by molding paraffin, bees wax, or the like, and a combustible solid, and inserting a wick into the center of the candle. In the case of lighting the wick, the candle positioned at the bottom of the wick is melted, and the melted candle rises upwardly along the wick by a capillary phenomenon to thereby be vaporized and combusted at a distal end portion of the wick, such that a flame burns. A combustion temperature of a surface flame of the candle is 1400° C. or more, a temperature of the brightest inner flame thereof is 1200° C. or more, and a temperature of a flame center thereof is 400 to 900° C.

The wick is generally used in material forms of a cotton wick, a wood wick, a zinc wick, a paper wick, etc. However, conventional candles into which wicks are inserted have unique problems as follows.

First, there is an excessive length amount of the remaining combusted wick. When an excessive length amount of the combusted wick remains, a flame size of the candle is increased, the candle burns much faster, and a large amount of soot due to combustion also occurs. Therefore, to control the flame size, it is inconvenient to periodically cut the wick or discard wax drippings from the candle. Further, in the case of the cotton wick, there is a case where a wick tip becomes bent after the candle is blown out, such that it is troublesome to cut the wick short before lighting the candle.

Second, there is a problem in that ash falls from the wick. When the ash of the wick falls, the candle is stained and looks dirty in view of aesthetics, and it is inconvenient to remove the ash.

In recent years, technologies for reducing soot and burning the wick properly at the time of combustion, such as a smokeless wick made of natural fibers, an eco wick, etc., have been developed. However, due to material limitations of the natural fibers, it is not enough to solve the above-described problems.

U.S. Patent Application Publication No. 2012-0148966 discloses a candle wick having a cross (+) shape in which the candle wick is perpendicularly oriented. In this case, the candle wick may be supported in an upright manner through the cross (+) shape, but problems of soot and ash still remain.

## 2

Korean Patent Publication No. 1492333 discloses a natural material candle wick produced from the heart of a stem of Stephanandra incise, and describes that incomplete combustion is able to be suppressed through the natural material candle wick. However, since hydrocarbon-based organic materials are used as a wick material, occurrence of soot and ash may still be a problem, and since physicochemical properties of the natural material are not uniform, and there is wide variation in amounts of soot and ash for each product. Therefore, there is a need to develop a technology in which a length of a wick remaining after combustion is able to be constantly maintained without causing the soot and ash.

15

## SUMMARY

An embodiment of the present invention is directed to providing a wick for a candle including a carbon material, wherein the carbon material is vaporized into carbon dioxide (CO<sub>2</sub>) gas at the time of combustion, such that a length of the wick is not longer than that of the conventional wick, and a phenomenon in which ash of the wick falls due to the combustion is remarkably reduced, and a candle including the wick for a candle.

Another embodiment of the present invention is directed to providing a wick for a candle in which carbon material is dispersed, wherein the carbon material is vaporized into carbon dioxide gas at the time of combustion, such that the length of the wick is not long, the phenomenon in which soot and ash of the wick fall is reduced, and a tunnel phenomenon in which the candle around the wick is melted down is improved, and a candle including the wick for a candle.

In one general aspect, there is provided a wick for a candle including a carbon material.

The carbon material may be any one or a mixture or a composite of two or more selected from carbon fiber, activated carbon, carbon nanotube, graphite, carbon black, graphene, graphene oxide, a carbon composite material, etc., but is not limited as long as the object of the present invention is achieved.

The carbon material may have a form of any one or two or more selected from long fibers, short fibers, fabrics and particles.

45 The wick may be selected from the following (i) to (v): (i) a wick formed of the carbon material alone, (ii) a wick in which the carbon material is dispersed in a matrix formed of any one selected from a binder and pulp, or a mixture thereof, (iii) a wick including the carbon material in a fabric formed of any one or two or more fibers selected from natural fibers and synthetic fibers, (iv) a wick including the carbon material in the fabric formed of any one or two or more fibers selected from natural fibers and synthetic fibers, the fabric being coated or impregnated with a binder, and (v) 50 a wick including the carbon material and any one or two or more short fibers selected from short fibers of natural fibers and short fibers of synthetic fibers, in the matrix formed of any one selected from a binder and pulp, or a mixture thereof.

55 The wick may have a web form including pores in the wick to allow fuel of the candle to be moved by a capillary phenomenon.

The wick for a candle may further include a supporter selected from a wood wick, a zinc wick, a tin wick, and a zinc-tin mixed metal wick.

60 The binder may have a melting temperature satisfying Equation 1 below:

melting temperature of fuel used in candle < melting temperature of binder. [Equation 1]

The wick may be coated with wax.

The wick for a candle may further include a wick clip.

In another general aspect, there is provided a candle including the wick for a candle as described above.

The candle may include any one or two or more fuels selected from paraffin wax, paraffin oil, soy wax, bees wax, palm wax, gel wax, etc.

The fuel may further include any one or two or more additives selected from fragrance and dye.

#### BRIEF DESCRIPTION OF THE DRAWINGS

FIG. 1 shows a candle including a plate-shaped wick 10a for a candle and a fuel 20 according to an exemplary embodiment of the present invention.

FIG. 2 shows a candle including a twisted wick 10b for a candle and a fuel 20 according to an exemplary embodiment of the present invention.

FIG. 3 shows a cross section of a straw-shaped wick woven with a diagonal mesh 10c according to an exemplary embodiment of the present invention.

FIG. 4 shows a cross section of a straw-shaped wick woven with a straight mesh 10d according to an exemplary embodiment of the present invention.

FIG. 5 shows a wick in which carbon material particles 200a are dispersed in a matrix formed of a binder according to an exemplary embodiment of the present invention.

FIG. 6 shows a wick in which carbon material short fibers 200b are dispersed in a matrix formed of a binder according to an exemplary embodiment of the present invention.

FIG. 7 shows a wick in which carbon material long fibers 200c are dispersed in a matrix formed of a binder according to an exemplary embodiment of the present invention.

FIG. 8 shows a wick in which carbon material particles 200a are dispersed in a matrix formed of pulp 200d.

FIG. 9 shows a wick in which carbon material short fibers 200b are dispersed in the matrix formed of pulp 200d.

FIG. 10 shows a wick in which carbon material long fibers 200c are dispersed in the matrix formed of pulp 200d.

FIG. 11 shows a wick in which carbon material particles 200a are dispersed in a fabric formed of fibers 200e.

FIG. 12 shows a wick in which carbon material short fibers 200b are dispersed in the fabric formed of fibers 200e.

FIG. 13 shows a wick in which carbon material long fibers 200c are dispersed in the fabric formed of fibers 200e.

FIG. 14 is an image of a sheet including a carbon material according to an exemplary embodiment of the present invention.

FIG. 15 is a front view showing a candle according to an exemplary embodiment of the present invention.

FIG. 16 is a side view showing a candle according to an exemplary embodiment of the present invention.

#### DETAILED DESCRIPTION OF MAIN ELEMENTS

10a: plate-shaped wick

10b: twisted wick

10c: straw-shaped wick woven with diagonal mesh

10d: straw-shaped wick woven with straight mesh

20: fuel

200a: carbon material particles dispersed in matrix

200b: carbon material short fibers dispersed in matrix

200c: carbon material long fibers dispersed in matrix

200d: matrix formed of pulp

200e: matrix formed of fiber

#### DETAILED DESCRIPTION OF EMBODIMENTS

5 Hereinafter, the present invention will be described in detail. The present invention may be specifically appreciated by the following Examples, and Examples below are given by way of illustration but are not intended to limit the protective scope defined by the attached claims of the present invention.

A content ratio or a mixing ratio used in the present invention is defined based on a weight of each component unless otherwise defined.

The inventors of the present invention found that when a wick for a candle includes a carbon material, the carbon material is directly vaporized into carbon dioxide (CO<sub>2</sub>) gas at the time of combustion of the wick, such that soot and ash rarely occur, and completed the present invention.

20 The present inventor also found that a tunnel phenomenon was able to be suppressed by dispersing the carbon material in a matrix forming the wick, and completed the present invention.

25 The wick for a candle according to the present invention preferably includes pores in the wick so that fuel of the candle is able to be moved to an upper end portion of the wick by a capillary phenomenon. When the pores are included, the fuel around the wick may be sucked up well and a flame size may be constantly maintained. Further, as the flame of the wick burns, the wick may burn together.

30 Hereinafter, an exemplary embodiment of the present invention is described in more detail.

An aspect of the present invention relates to a wick for a candle including a carbon material.

35 In the present invention, the carbon material is a material in which at least 90% constituent atoms are carbon atoms, and thermal resistance, durability and conductivity are excellent due to bonds between carbon and carbon.

40 In an exemplary embodiment of the present invention, a carbon content of the carbon material is preferably 40 to 100 wt %, more preferably 50 to 100 wt %, based on the total weight of the wick, in order to exhibit an effect of reduced soot and a rare occurrence of ash due to the carbon material, but the carbon content is not limited thereto. That is, when the carbon content is less than 40 wt %, even though the degree of the effect may be reduced, the effect may be exhibited, and thus, the carbon content may be controlled as needed.

45 In an exemplary embodiment of the present invention, the carbon material may be any one or a mixture or a composite of two or more selected from carbon fiber, activated carbon, carbon nanotube, graphite, carbon black, graphene, graphene oxide, a carbon composite material, etc.

50 As a specific example, when the carbon material is the carbon fiber, the carbon material may be any one or two or more selected from rayon-based carbon fiber, PAN-based carbon fiber, pitch-based carbon fiber, etc., but is not limited thereto.

55 The carbon composite material is a material having improved mechanical strength as compared to conventional carbon fibers. For example, the carbon composite material may be a carbon-carbon composite material obtained by impregnating the carbon fiber with a phenolic resin, followed by carbonization and graphitization at a high temperature of 1000 to 2500° C. to increase strength, a silicon carbide (SiC) composite material obtained by using poly-carbosilane which is an organic silicon polymer as a pre-

cursor, followed by sintering at 800 to 1200° C., or the like, but the present invention is not limited thereto.

According to an exemplary embodiment of the present invention, the carbon material may have a form of any one or two or more selected from long fibers, short fibers, fabrics and particles, and may be included as carbon material dispersion bodies in the wick.

More specifically, an exemplary embodiment of the present invention provides a wick for a candle including a carbon material which is vaporized into carbon dioxide at the time of combustion of the wick wherein pores are included in the wick to allow fuel of the candle to be moved by a capillary phenomenon, and the carbon material is dispersed in a matrix forming the wick.

In an exemplary embodiment of the present invention, the carbon material long fiber may be a long fiber formed of carbon fiber, activated carbon, carbon nanotube, graphite, carbon black, graphene, graphene oxide, a carbon composite material, etc., as described above. A length of the long fiber is not particularly limited as long as it is able to form the wick. As a non-limiting example, the long fiber may have a diameter of 0.01 to 50  $\mu\text{m}$ , preferably of 0.1 to 20  $\mu\text{m}$ . When the above-described range is satisfied, it may be advantageous to produce a fabric including pores, etc.

The carbon material short fiber has an average fiber length shorter than that of the long fiber. As a non-limiting example, the carbon material short fiber may have a diameter of 0.01 to 50  $\mu\text{m}$ , preferably 0.1 to 20  $\mu\text{m}$ , and an average length of 0.01 to 25 mm, preferably 0.1 to 20 mm, and more preferably 1 to 10 mm, but these are not particularly limited as long as it is within a range satisfying physical properties used for the wick. When the above-described range is satisfied, since the carbon material short fibers are well dispersed, the carbon material short fibers may be uniformly mixed with a binder, or the like.

The carbon material fabric may be produced by weaving or electrospinning the carbon material. More specifically, the carbon material fabric may be produced by weaving the carbon material long fiber, or may be woven by mixing the carbon material long fiber with other fibers. In addition, the carbon material fabric may be produced by electrospinning a spinning solution including carbon fiber, activated carbon, carbon nanotube, graphite, carbon black, graphene, graphene oxide, a carbon composite material, etc., and when the carbon material fabric is produced by electrospinning, the carbon material fabric may have a web form including pores with dense micropores formed therein. The electrospinning is not limited as long as it is a method known in the art, and for example, Korean Patent No. 10-1392227, Korean Patent Laid-Open Publication No. 10-2016-0000112, Korean Patent Laid-Open Publication No. 10-2013-0073481, Korean Patent No. 10-0783490, Korean Patent No. 10-1370867, etc., may be referred.

The carbon material particles may be particles of carbon fiber, activated carbon, carbon nanotube, graphite, carbon black, graphene, graphene oxide, a carbon composite material, etc. The 'particle' refers to powder having a finer diameter than that of the short fiber. The carbon material particles may have an average particle diameter of 10 to 5000 nm, preferably 100 to 3000 nm, but the average particle diameter thereof is not particularly limited as long as it is intended to form the wick. When the average particle diameter satisfies the above-described range, it is preferred since the carbon material particles have good dispersibility.

In the present invention, a direction in which the wick is combusted is referred to as a "length direction".

In an aspect of the present invention, in consideration of a shape and a size of the candle to be designed, a length of the wick for a candle with respect to the length direction, and an average diameter or a width of the wick for a candle may be controlled. As an example, the length may be 1 to 50 cm, preferably 3 to 30 cm, and more preferably 5 to 15 cm with respect to the length direction of the wick, but is not limited thereto. In addition, the average diameter or the width of the wick may be 0.01 to 100 mm, preferably 0.1 to 50 mm, and more preferably 0.5 to 20 mm, but is not limited thereto.

Hereinafter, the wick for a candle including the carbon material according to the present invention will be described in detail with reference to the drawings. The accompanying drawings are exemplified to describe an exemplary embodiment of the present invention. The present invention is not limited thereto.

The wick for a candle in the present invention may be a plate-shaped wick 10a as shown in FIG. 1, a twisted wick 10b as shown in FIG. 2, and straw-shaped wicks 10c and 10d as shown in FIGS. 3 and 4, but is not limited thereto.

Specifically, FIG. 1 shows a candle including a plate-shaped wick 10a and a fuel 20 according to an exemplary embodiment of the present invention. FIG. 2 shows a candle including a twisted wick 10b and a fuel 20 according to an exemplary embodiment of the present invention. At this time, the twisted shape may be produced by crossing two or more fiber bundles as shown in FIG. 2. FIGS. 3 and 4 show cross sections of the straw-shaped wicks 10c and 10d according to an exemplary embodiment of the present invention. The straw shape means that an inside of a cylinder is empty. FIG. 3 shows the straw-shaped wick woven with a diagonal mesh 10c and FIG. 4 shows the straw-shaped wick woven with a straight mesh 10d.

The wick for a candle as shown in FIGS. 1 to 4 in an exemplary embodiment of the present invention may be selected from the following (i) to (v): (i) a wick formed of the carbon material alone, (ii) a wick in which the carbon material is dispersed in a matrix formed of any one selected from a binder and pulp, or a mixture thereof, (iii) a wick including the carbon material in a fabric formed of any one or two or more fibers selected from natural fibers and synthetic fibers, (iv) a wick including the carbon material in the fabric formed of any one or two or more fibers selected from natural fibers and synthetic fibers, the fabric being coated or impregnated with a binder, and (v) a wick including the carbon material and any one or two or more short fibers selected from short fibers of natural fibers and short fibers of synthetic fibers, in the matrix formed of any one selected from a binder and pulp, or a mixture thereof.

More specifically, (i) the wick formed of the carbon material alone is described.

The carbon material according to the (i) exemplary embodiment may be any one or a mixture or a composite of two or more selected from carbon fiber, activated carbon, carbon nanotube, graphite, carbon black, graphene, graphene oxide, and a carbon composite material, and the carbon material may have a long fiber form or a fabric form. Specifically, for example, the wick may be a twisted wick made by twisting long fibers formed of the carbon material into several strands. The twisted wick may have the same shape as the wick 10b shown in FIG. 2, but is not limited thereto. In addition, the wick may be the straw-shaped wicks (10c and 10d) made by weaving a fabric including the carbon material into a straw shape as shown in FIGS. 3 and 4. In addition, the wick may be produced by cutting the fabric including the carbon material into the plate shape 10a as shown in FIG. 1. Further, the wick may be the straw-

shaped wicks (10c and 10d) made by rolling the fabric including the carbon material as shown in FIGS. 3 and 4.

Next, the (ii) wick in which the carbon material is dispersed in a matrix formed of any one selected from a binder and pulp, or a mixture thereof will be described.

In the (ii) exemplary embodiment, the carbon material having a form of any one or two or more selected from long fibers, short fibers, fabrics and particles may be included in the matrix as a dispersion body. The shape of the wick may be one of the shapes of FIGS. 1 to 4 as described above, but is not limited thereto. When the wick has a plate shape as shown in FIG. 1, the wick may be produced by conventional methods such as spin coating, bar coating, casting, etc., which is not limited to the above-exemplified methods as long as the plate-shaped article may be produced. As shown in FIG. 2, the twisted wick may be produced by cutting the wick formed in a plate form, twisting the wicks, or twisting a plurality of strands of long fiber bundles.

In the (ii) exemplary embodiment, it is preferable to use a matrix material having a low thermal conductivity as the matrix material since high thermal conductivity of the carbon material is reduced to prevent the tunnel phenomenon from occurring. As the carbon material dispersion bodies are dispersed in the matrix, thermal transfer between the carbon material dispersion bodies is reduced and thermal transfer of the matrix material is not performed well, which is more preferred to prevent the tunnel phenomenon in which the fuel of the candle melts around the wick. More preferably, the carbon material dispersion bodies may be spatially spaced apart from each other in the matrix to further reduce thermal transfer.

As a non-limiting example, the matrix material may have thermal conductivity less than 1 W/m·K, preferably less than 0.4 W/m·K, more preferably between 0.01 to 0.2 W/m·K, which is preferred to suppress the tunnel phenomenon.

As a specific example, in the (ii) exemplary embodiment, a case where the matrix is formed of a binder will be described.

In the (ii) exemplary embodiment, the wick may be a wick in which carbon materials in a form of particles are dispersed in a matrix formed of a binder, a wick in which carbon materials in a form of short fibers are dispersed in the matrix formed of a binder, and a wick in which carbon materials in a form of long fibers are dispersed in the matrix formed of a binder.

More specifically, dispersion of the carbon materials is shown in FIGS. 5 to 7. Referring to the drawings, FIG. 5 shows a wick in which carbon material particles 200a are dispersed in the matrix formed of the binder. FIG. 6 shows a wick in which carbon material short fibers 200b are dispersed in the matrix formed of the binder. FIG. 7 shows a wick in which carbon material long fibers 200c are dispersed in the matrix formed of the binder.

In an exemplary embodiment of the present invention, the binder may have a melting temperature satisfying Equation 1 below, which may be applied in the same way in all the following exemplary embodiments.

$$\text{melting temperature of fuel used in candle} < \text{melting temperature of binder.} \quad [\text{Equation 1}]$$

When the melting temperature of the binder is higher than that of the fuel, it is preferable since the binder of the wick is not melted and the shape of the wick is able to be maintained as it is. When the melting temperature of the fuel used in the candle is equal to or higher than that of the

binder, the binder of the wick may melt due to a temperature of a molten fuel, and the wick may not be maintained in a straight shape.

In an exemplary embodiment of the present invention, the fuel used in the candle may include any one or two or more fuels selected from paraffin wax, soy wax, bees wax, gel wax, etc. The fuel may have a melting temperature of 40 to 70° C.

Further, the binder may include any one or a mixture of two or more selected from a polyamide-based resin, a polyvinyl-based resin, a polyolefin-based resin, a polyester-based resin, an acrylate-based resin, a cellulose-based resin, an epoxy resin, a phenol-based resin, etc., but is not limited thereto. More specifically, the binder may be any one or a mixture of two or more selected from polyvinyl alcohol, polyvinyl pyrrolidone, polyvinyl butyral, polyvinyl acetate, low density polyethylene, linear low density polyethylene, medium density polyethylene, high density polyethylene, polypropylene, ethylene vinyl acetate resin, poly isoprene, nylon 6, nylon 66, polyethylene carbonate, polypropylene polycarbonate, bisphenol A-polycarbonate, polyethylene terephthalate, polybutylene terephthalate, polymethyl methacrylate, methylcellulose, carboxymethylcellulose, epoxy resin, phenol-formaldehyde resin, paraffin, etc.

When the paraffin is used as a binder in an exemplary embodiment of the present invention, the fuel used in the candle may be a fuel having a lower melting temperature than that of paraffin, such as soy wax, etc.

Next, in the (ii) exemplary embodiment, a case where the matrix is formed of pulp will be described.

In the (ii) exemplary embodiment, the wick may be a wick in which carbon materials in a form of particles are dispersed in a matrix formed of pulp, a wick in which carbon materials in a form of short fibers are dispersed in the matrix formed of pulp, and a wick in which carbon materials in a form of long fibers are dispersed in the matrix formed of pulp.

More specifically, dispersion of the carbon materials is shown in FIGS. 8 to 10. Referring to the drawings, FIG. 8 shows a wick in which carbon material particles 200a are dispersed in a matrix formed of pulp 200d. FIG. 9 shows a wick in which carbon material short fibers 200b are dispersed in the matrix formed of pulp 200d. FIG. 10 shows a wick in which carbon material long fibers 200c are dispersed in the matrix formed of pulp 200d.

In the present invention, the matrix formed of pulp may maintain a shape and strength of the wick, and twigs of cellulose-based fibers may physically and stably fix the carbon material. At this time, the pulp may be a cellulose-based fiber produced by mechanical pulverization, or by pressure, heat, or chemical treatment of wood or plant fibers.

The pulp is a cellulose-based fiber which is fibrillated to include a number of twigs through mechanical or chemical treatment, wherein a stem branch of the fiber has a diameter of several tens of micrometers (μm), but the twigs connected to the stem branch have a diameter of several micrometers and are complexly connected to each other, and preferably may have a three-dimensional mesh structure. Due to the three-dimensional mesh structure, the pulp and the carbon material particles, the short fibers or the long fibers may be physically coupled to each other or entangled with each other and may be dispersed in a stable form in the mesh structure of the pulp without special treatment to form a wick having high porosity.

As a non-limiting specific example, the pulp may be wood pulp such as hardwood such as birch, eucalyptus, oak, etc., and softwood such as pine, fir, etc., or non-wood pulp

including plant fiber such as straw, cotton, bark of paper mulberry, etc., as raw materials.

As a non-limiting example, the pulp may have an average fiber length of 0.1 to 20 mm, preferably 0.5 to 10 mm. When the average fiber length of the pulp satisfies the above-described range, it is preferable in that the shape and strength of the wick may be maintained, and the twigs of the cellulose-based fiber may fix the carbon material physically and stably.

In addition, in the (ii) exemplary embodiment, a case where the matrix is formed of a mixture of a binder and pulp will be described.

In the (ii) exemplary embodiment, when the mixture of the binder and pulp is used as the matrix, a mixing ratio of the binder and the pulp may be a weight ratio of 1:9 to 9:1, preferably 2:8 to 4:6, but is not limited thereto. When the mixing ratio satisfies the above-described range, it is preferred that the binder and the pulp may be effectively mixed, rigidity of the fibers included in the pulp may be further improved by the binder, and thus rigidity of the wick may be improved to maintain the shape of the wick. Further, the carbon material is strongly coupled by the binder, and the carbon material coupled by the binder is fixed to the twigs of the cellulose-based fiber present in the pulp, which may be particularly preferable in that it is possible to have a high porosity and a strong binding strength.

As a specific example, a mixing ratio of any one selected from the binder and the pulp or a mixture thereof and the carbon material may be a weight ratio of 10:90 to 90:10, more preferably a weight ratio of 15:85 to 85:15, and more preferably 45:55 to 55:45, but is not limited thereto. When the mixing ratio satisfies the above-described range, it is preferred that the carbon material may be fixed in the matrix to thereby prevent the carbon material from being separated, to maintain the shape of the wick, and to effectively suppress formation of soot and ash due to a high carbon material content.

As a non-limiting example, the wick according to the (ii) exemplary embodiment may be formed of a plate-shaped sheet including carbon material short fibers, pulp and a binder, wherein the pulp is a fibrillated cellulose-based fiber having a three-dimensional mesh structure, and the carbon material short fibers may be dispersed in the wick.

Next, (iii) the wick including the carbon material in fabric formed of any one or two or more fibers selected from natural fibers and synthetic fibers will be described.

The wick of the (iii) exemplary embodiment may be produced in a plate shape, a twisted shape and a straw shape as shown in FIGS. 1 to 4, but the shape of the wick is not limited thereto.

In the (iii) exemplary embodiment, the natural fiber may be any one or two or more mixed fibers selected from cotton, hemp, silk, wool, etc., but is not limited thereto. The synthetic fiber may be any one or two or more mixed fibers selected from polyamide-based fiber, polyolefin-based fiber, polyester-based fiber, polyvinyl alcohol-based fiber, polyacrylate-based fiber and polyurethane fiber, etc., and may be a copolymer fiber produced through copolymerization with a comonomer. Preferably, the fiber may be nylon 6 fiber, nylon 66 fiber, polyethylene fiber, polypropylene fiber, polyethylene terephthalate fiber, polybutylene terephthalate fiber, polyvinyl alcohol fiber, polyacrylonitrile fiber, poly(vinyl chloride-co-acrylonitrile) or butanediol-derived polyurethane fiber, etc., but is not limited thereto.

In the (iii) exemplary embodiment, the carbon material included in the fabric may have a form of any one or two or more selected from long fibers, short fibers, fabrics and particles.

5 An exemplary embodiment thereof is shown in FIGS. 11 to 13. Referring to the drawings, FIG. 11 shows a wick in which carbon material particles 200a are dispersed in a fabric 200e formed of any one or two or more fibers selected from natural fibers and synthetic fibers. FIG. 12 shows a 10 wick in which the carbon material short fibers 200b are dispersed in the fabric 200e. FIG. 13 shows a wick in which the carbon material long fibers 200c are dispersed in the fabric 200e. In FIG. 13, the fabric may be produced by 15 weaving the carbon material in a long fiber form and any one or two or more fibers selected from natural fibers and synthetic fibers.

In the (iii) exemplary embodiment, the dispersion may be performed by blowing at high pressure or by spraying to 20 physically fix the carbon material. Preferably, it is particularly preferable to disperse the carbon material particles or the carbon material short fibers on a surface of the fiber by blowing or spraying, followed by annealing at a glass transition temperature or higher of the polymer constituting 25 the fiber for a predetermined time to perform physical binding, and thus, the carbon material particles or the carbon material short fibers may have strong binding strength without being separated from the fiber. Time for annealing may be at least 2 minutes, preferably 5 minutes to 60 30 minutes, but may vary depending on the type and diameter of the fiber, and is not limited thereto.

In the (iii) exemplary embodiment, a content of the carbon material may be 50 to 90 wt %, preferably 55 to 85 wt % based on the total weight of the wick, but is not particularly 35 limited as long as the object of the present invention is achieved. When the content thereof satisfies the above-described range, it is preferable since it is possible to minimize soot and ash of the wick at the time of combustion.

Next, (iv) the wick including the carbon material in the 40 fabric formed of any one or two or more fibers selected from natural fibers and synthetic fibers, the fabric being coated or impregnated with a binder will be described.

The wick of the (iv) exemplary embodiment may be produced in a plate shape, a twisted shape and a straw shape 45 as shown in FIGS. 1 to 4, but the shape of the wick is not limited thereto.

Further, the wick may be a wick in which the wick of the (iii) exemplary embodiment shown in FIGS. 11 to 13 is applied or impregnated with a binder, and further drawings 50 thereof are not provided.

In the (iv) exemplary embodiment, it is preferable that a content of the binder may be preferably 1 to 20 parts by weight, and more preferably 5 to 15 parts by weight, based on 55 100 parts by weight of the fabric including the carbon material. By further applying or impregnating the wick with the binder, the rigidity of the wick may be further improved, and the carbon material physically fixed to the surface of the fiber may be coupled more strongly by the application or impregnation of the binder.

60 The (iv) exemplary embodiment is preferable in that it is possible to have porosity due to the distance between fibers and to have a strong binding strength by the binder at the same time. Here, the binder may have the same components as the above-described binder.

65 The method of applying or impregnating in the (iv) exemplary embodiment is not particularly limited, but may include a spray coating method, a dip coating method, a

## 11

painting method, etc., known in the art, and is not limited as long as it is a method of applying the surface of the fiber with a binder.

Next, (v) the wick including the carbon material and any one or two or more short fibers selected from short fibers of natural fibers and short fibers of synthetic fibers, in the matrix formed of any one selected from a binder and a pulp, or a mixture thereof will be described.

The wick of the (v) exemplary embodiment may be produced in a plate shape, a twisted shape and a straw shape as shown in FIGS. 1 to 4, but the shape of the wick is not limited thereto.

In the (v) exemplary embodiment, the wick may further include any one or two or more short fibers selected from short fibers of natural fibers and short fibers of synthetic fibers when producing the wick of the (ii) exemplary embodiment, and separate drawings are omitted.

The (v) exemplary embodiment will be described in detail. The wick may be a wick in which carbon material particles and short fibers of natural fibers are dispersed in a matrix formed of a binder, a wick in which carbon material short fibers and the short fibers of natural fibers are dispersed in the matrix formed of a binder, and a wick in which carbon material long fibers and the short fibers of natural fibers are dispersed in the matrix formed of a binder. In addition, the wick may be a wick in which carbon material particles and short fibers of natural fibers are dispersed in a matrix formed of pulp, a wick in which carbon material short fibers and the short fibers of natural fibers are dispersed in the matrix formed of pulp, and a wick in which carbon material long fibers and the short fibers of natural fibers are dispersed in the matrix formed of pulp.

In the (v) exemplary embodiment, any one or two or more short fibers selected from the short fibers of the natural fibers and the short fibers of synthetic fibers are used in a content of 0.1 to 20 parts by weight, preferably 1 to 10 parts by weight, based on 100 parts by weight of the wick of the (ii) exemplary embodiment, but the content is not particularly limited as long as the object of the invention is achieved. When the content thereof satisfies the above-described range, it is preferable since it is possible to maximize the porosity while minimizing soot and ash of the wick at the time of combustion.

In the (v) exemplary embodiment, the short fibers of the natural fibers and the short fibers of the synthetic fibers may preferably have an average length of 0.01 to 25 mm, preferably 0.1 to 20 mm, and more preferably 1 to 10 mm. Within the above-described range, the fibers may be effectively dispersed in the matrix together with the carbon material. By including the short fibers of the natural fibers or the synthetic fibers in the matrix, the porosity of the wick may be further improved and the porosity per unit volume of the wick may be improved.

According to an exemplary embodiment of the present invention, it is preferred that the wick for a candle has a web form including pores in the wick so that the fuel of the candle may be moved to the upper end portion of the wick by a capillary phenomenon. Here, the fuel of the candle may be a fuel in which a solid fuel of the candle is melted to be a liquid state at the time of combustion, or a liquid fuel such as paraffin oil, or the like. The wick may allow the molten solid fuel or liquid fuel of the candle to be moved to the upper end portion of the wick by a capillary phenomenon. The web form means that the fibers or particles are entangled with each other to include pores. Since there are a number of fine pores of the wick, heat shielding performance may be

## 12

excellent to reduce thermal conductivity of the carbon material included in the wick.

It is preferable that the pores of the wick may have a porosity of 40 to 90 wt %, preferably 50 to 80 wt %, based on the total volume of the entire wick. In addition, as an example, the pores of the wick may have a size of 1 nm to 1000  $\mu\text{m}$ , preferably 100 nm to 500  $\mu\text{m}$  in diameter. When the size of the pores of the wick satisfies the above-described range, a physical form of the wick may be maintained, thermal conductivity of the wick may be reduced, and the fuel of the candle may be moved by the capillary phenomenon at the time of combustion of the candle, thereby maintaining flame.

According to an exemplary embodiment of the present invention, the wick for a candle may further include a supporter selected from a wood wick, a zinc wick, a tin wick, a zinc-tin mixed metal wick, etc. Preferably, the use of the zinc wick is safe at the time of combustion, and is preferable in that since zinc may be vaporized within a flame temperature, but it is not particularly limited as long as the object of the present invention is achieved. When the supporter is included, it is possible to prevent the wick from being bent when the tunnel phenomenon occurs due to melting of the fuel of the candle at the time of combustion.

Regarding the supporter, at least one supporter may be inserted into the inside of the wick, or at least any one supporter may be coupled to at least one surface of the wick. Here, the wick may further include an adhesive. The adhesive may increase a binding strength between the wick and the supporter. The adhesive may have the same component as the above-described binder.

For example, the supporter may have a plate shape, a strip shape, a flat plate strip shape, a wire shape, a bar shape, etc. Specifically, the wood wick may have a strip shape, a flat plate strip shape and a bar shape, and the zinc, tin and zinc-tin mixed metal wick may have a wire shape.

As a specific example, a wire-shaped zinc wick supporter may be inserted into the inside of the twisted wick, or a plate-shaped wood wick supporter may be coupled with the plate-shaped wick, wherein a coupled configuration may be made in the manner in which surface-to-surface of the plates is coupled in the same length direction as the length direction of the wick, but is not limited thereto.

In addition, the supporter may have an appropriate length in consideration of the shape and size of the wick to be designed. As an example, the length of the supporter may be 1 to 50 cm, preferably 5 to 30 cm, and more preferably 5 to 15 cm, but is not limited thereto. In addition, the average diameter or width of the supporter may be 0.001 to 50 mm, specifically 0.1 to 10 mm, but is not limited thereto.

According to an exemplary embodiment of the present invention, the wick for a candle may be coated with wax. As a specific example, the coating may be performed by using any one method selected from dip coating in which the wick is immersed into a molten wax, dry coating, laminating, spraying methods, and the like. The method for coating is not limited as long as it is any coating method known in the art.

As a specific example, the wax may be any one or a mixture of two or more selected from paraffin wax, bees wax, soy wax, palm wax, gel wax, etc., but is not limited thereto.

The wick coated with wax may allow initial ignition of the wick to be effectively generated by using the wax as fuel at the time of combustion. Further, the wick coated with wax is preferable in that it is possible to maintain a stiff and

## 13

straight state, and to prevent the tunnel phenomenon due to thermal transfer at the time of combustion.

According to an exemplary embodiment of the present invention, the wick may further include a wick clip. The wick clip may fix the wick vertically. A shape of the wick clip is not particularly limited, and may be various shapes such as circle, triangle, square, a clip shape, etc., depending on the purpose.

According to another embodiment of the present invention, there is provided a candle including the wick. In the present invention, the candle may include a fuel. The fuel may be a solid fuel or a liquid fuel. Here, the fuel may enclose the wick of the candle. A position of the wick is not particularly limited, but it is preferable that the wick is positioned at the center of the candle. When the wick is positioned at the center of the candle, it is preferable in that a flame of the wick may uniformly melt the fuel at the time of combustion of the candle. The fuel of the candle may be raised by the capillary phenomenon of the wick, thereby maintaining the combustion of the wick.

As a specific example, the fuel of the candle may be any one or a mixture of two or more selected from paraffin wax, paraffin oil, bees wax, soy wax, palm wax, gel wax, etc., but is not limited thereto.

According to the exemplary embodiment of the present invention, the fuel of the candle may further contain one or two or more additives selected from perfumes and dyes. It is preferred that the perfume and the dye are not harmful to the human body.

A specific example of the perfume may include fragrance oil corresponding to artificial perfume and/or natural essential oil extracted from plant, but is not limited thereto. As a more specific example, the perfume may be one or two or more selected from perfumes of lavender, rosemary, jasmine, chamomile, rose, geranium, lily, daisy, lemon, cinnamon, eucalyptus, bergamot, peach, etc.

As a specific example, the perfume may be included in a content of 0.1 to 10 parts by weight, preferably, 1 to 5 parts by weight, based on 100 parts by weight of the candle, but is not limited thereto. When the content of the perfume satisfies the above-described range, it is preferred since the candle may emit subtle fragrance at the time of combustion.

The dye is not particularly limited, but a dye having a suitable color may be selected depending on the object. As an example, the dye is a dye for a candle that is not harmful. As a specific example, the dye may have one or two or more colors selected from red, yellow, green, orange, purple, pink, brown, etc.

As a specific example, the dye may be contained in a content of 0.1 to 10 parts by weight, preferably, 1 to 5 parts by weight, based on 100 parts by weight of the candle (the fuel of the candle), but is not limited thereto. When the content of the dye satisfies the above-described range, it is preferred since a color of the candle may be exhibited.

According to the exemplary embodiment of the present invention, the candle may have various sizes and shapes depending on the object, and is not particularly limited. As a specific example, the candle may have any one or two or more selected from a cylindrical shape, a tetragonal shape, a triangular shape, a pentagonal shape, a hexagonal shape, a heart shape, a star shape, etc.

Hereinafter, the carbon material wick for a candle and the candle including the same according to the present invention will be described in more detail through Examples. However, the following Examples are only references for spe-

## 14

cifically explaining the present invention, but the present invention is not limited thereto and may be implemented in various forms.

In addition, unless defined otherwise, all technical and scientific terms used herein have the same meanings generally understood by those skilled in the art to which the present invention pertains. Terms used in the specification of the present invention are to effectively describe specific exemplary embodiments, but are not intended to limit the present invention.

In addition, the drawings to be described below are provided by way of example so that the idea of the present invention can be sufficiently transferred to those skilled in the art to which the present invention pertains. Therefore, the present invention may be implemented in many different forms, without being limited to the drawings to be described below. The drawings to be provided below may be exaggerated in order to specify the spirit of the present invention.

It is intended that singular forms used in the specification and claims include plural forms unless otherwise indicated in the context.

## EXAMPLE 1

40 wt % of an aqueous solution containing 50 wt % of 25 polyvinyl alcohol (Sigma-Aldrich Co., weight average molecular weight of 31,000 to 50,000 g/mol, 98 to 99% hydrolyzed, melting point of 200° C.) was mixed with 60 wt % of wood pulp having an average length of 5 mm.

70 wt % of the mixture was mixed with 30 wt % of short 30 fibers of activated carbon fiber having an average length of 3 mm, followed by casting on a flat plate with a frame to manufacture a sheet having a thickness of 0.3 mm. The manufactured sheet was dried at 25° C. for 36 hours. The dried sheet was cut into a size of 2 mm×7 cm (width×length) 35 to produce a wick. After melting paraffin wax having a melting point of 61° C. by raising a temperature to the melting point, the wick was immersed in the melted solution to coat the paraffin wax on a surface of the wick.

70 wt % of the mixture was mixed with 30 wt % of short 40 fibers of activated carbon fiber having an average length of 3 mm, followed by casting on a flat plate with a frame to manufacture a sheet having a thickness of 0.3 mm. The manufactured sheet was dried at 25° C. for 36 hours. The dried sheet was cut into a size of 2 mm×7 cm (width×length) 45 to produce a wick. After melting paraffin wax having a melting point of 61° C. by raising a temperature to the melting point, the wick was immersed in the melted solution to coat the paraffin wax on a surface of the wick.

A wick clip was inserted into one side of the coated wick,

40 and the wick was put into a heat resistant glass bottle having a diameter of 7 cm and a length of 8.5 cm. The wick was placed perpendicular to the bottom of a glass bottle.

200 g of paraffin wax having a melting point of 61° C. was warmed, and then placed in a glass container to produce a

45 candle having a height of 6.5 cm. The candle was allowed to stand at 25° C. for 24 hours to thereby be completely hardened and the wick of the candle was cut into a size of 5 mm to produce a candle.

## EXAMPLE 2

A candle was produced in the same manner as in Example 1 except that 50 wt % of the mixture was mixed with 50 wt % of the short fibers of activated carbon fiber having an 55 average length of 3 mm.

## EXAMPLE 3

A candle was produced in the same manner as in Example 60 1 except that 10 wt % of the mixture was mixed with 90 wt % of the short fibers of activated carbon fiber having an average length of 3 mm.

## EXAMPLE 4

The sheet of Example 1 was cut into a size of 1 mm×20 cm (width×length), and three cut strands were twisted at

## 15

regular intervals as shown in FIG. 2, thereby producing a twisted wick. The wick had a diameter of 2 mm and a length of 7 cm. The wick was coated with paraffin wax in the same manner as in Example 1, and then a candle was produced.

## EXAMPLE 5

A sheet cut into a size of 1 mm×50 cm (width×length) from the sheet of Example 1 was wound diagonally on a wooden bar having a diameter of 2 mm and wound one more time in the other direction, thereby producing a diagonal shaped fabric as shown in FIG. 3. Then, the fabric was immersed in an aqueous solution containing 50 wt % of polyvinyl alcohol (Sigma-Aldrich Co., weight average molecular weight 31,000 to 50,000 g/mol, 98 to 99% hydrolyzed, melting point of 200° C.), based on 100 parts by weight of the mixture, followed by casting on a flat plate with a frame to manufacture a sheet having a thickness of 0.3 mm. The manufactured sheet was dried at 25° C. for 36 hours. The dried sheet was cut into a size of 2 mm×7 cm (width×length) to produce a wick. After melting paraffin wax having a melting point of 61° C. by raising a temperature to the melting point, the wick was immersed in the melted solution to coat the paraffin wax on a surface of the wick.

5 of the short fibers of natural fibers of cotton having an average diameter of 100 µm and an average length of 10 mm were added and mixed with 20 parts by weight of an aqueous solution containing 50 wt % of polyvinyl alcohol (Sigma-Aldrich Co., weight average molecular weight of 31,000 to 50,000 g/mol, 98 to 99% hydrolyzed, melting point of 200° C.), based on 100 parts by weight of the mixture, followed by casting on a flat plate with a frame to manufacture a sheet having a thickness of 0.3 mm. The manufactured sheet was dried at 25° C. for 36 hours. The dried sheet was cut into a size of 2 mm×7 cm (width×length) to produce a wick. After melting paraffin wax having a melting point of 61° C. by raising a temperature to the melting point, the wick was immersed in the melted solution to coat the paraffin wax on a surface of the wick.

10 A candle was produced in the same manner as in Example 1 by using the wick.

## EXAMPLE 6

Natural fibers of cotton having an average diameter of 30 µm and rayon-based carbon fibers having an average diameter of 20 µm were mixed at a weight ratio of 1:1 to produce a fabric. The fabric was cut into a size of 2 mm×7 cm (width×length) to produce a wick. After melting paraffin wax having a melting point of 61° C. by raising a temperature to the melting point, the wick was immersed in the melted solution to coat the paraffin wax on a surface of the wick. A candle was produced in the same manner as in Example 1 by using the wick.

15 A candle was produced by using a zinc wick having a diameter of 0.5 mm and a length of 7 cm as a core while using the wick of Example 3, and the produced wick had a diameter of 2.5 mm. All processes were performed in the same manner as in Example 1, except that the wick as produced above was used.

## EXAMPLE 7

Fiber bundles obtained by mixing natural fibers of cotton having an average diameter of 30 µm and pitch-based carbon fibers having an average diameter of 30 µm at a weight ratio of 1:1 were twisted at regular intervals to produce a twisted wick as shown in FIG. 2. The wick was coated with paraffin wax in the same manner as in Example 1, and then a candle was produced.

20 30 parts by weight of an aqueous solution containing 50 wt % of polyvinyl alcohol (Sigma-Aldrich Co., weight average molecular weight of 31,000 to 50,000 g/mol, 98 to 99% hydrolyzed, melting point of 200° C.) was added and mixed with respect to 100 parts by weight of the short fibers of activated carbon fiber having an average length of 3 mm, followed by casting on a flat plate with a frame to manufacture a sheet having a thickness of 0.3 mm. The manufactured sheet was dried at 25° C. for 36 hours. The dried sheet was cut into a size of 2 mm×7 cm (width×length) to produce a wick. After melting paraffin wax having a melting point of 61° C. by raising a temperature to the melting point, the wick was immersed in the melted solution to coat the paraffin wax on a surface of the wick.

25 A candle was produced in the same manner as in Example 1 by using the wick.

## EXAMPLE 8

Natural fibers of cotton having an average diameter of 30 µm and rayon-based carbon fibers having an average diameter of 20 µm were mixed at a weight ratio of 1:1 to produce a fabric. The fabric was cut into a size of 2 mm×7 cm (width×length) to produce a wick.

30 35 40 45 As a result of combustion of the wick of the produced candle, soot and ash did not occur within 2 hours after the combustion, and the wick was combusted down together with the flame, but the combustion was not possible after 2 hours or longer due to the tunnel phenomenon in which the candle around the wick was melted down.

## COMPARATIVE EXAMPLE 1

All processes were performed in the same manner as in Example 1, except that a cotton wick (No. 3, Korea) was used as the wick.

## COMPARATIVE EXAMPLE 2

50 55 60 All processes were performed in the same manner as in Example 1, except that a smokeless wick (No. 3, Korea) was used as the wick.

## COMPARATIVE EXAMPLE 3

65 A wood wick having a thickness of 1 mm, a width of 1 cm and a length of 7 cm was inserted into a wick clip and used

## EXAMPLE 9

70 75 80 85 90 95 100 105 110 115 120 125 130 135 140 145 150 155 160 165 170 175 180 185 190 195 200 205 210 215 220 225 230 235 240 245 250 255 260 265 270 275 280 285 290 295 300 305 310 315 320 325 330 335 340 345 350 355 360 365 370 375 380 385 390 395 400 405 410 415 420 425 430 435 440 445 450 455 460 465 470 475 480 485 490 495 500 505 510 515 520 525 530 535 540 545 550 555 560 565 570 575 580 585 590 595 600 605 610 615 620 625 630 635 640 645 650 655 660 665 670 675 680 685 690 695 700 705 710 715 720 725 730 735 740 745 750 755 760 765 770 775 780 785 790 795 800 805 810 815 820 825 830 835 840 845 850 855 860 865 870 875 880 885 890 895 900 905 910 915 920 925 930 935 940 945 950 955 960 965 970 975 980 985 990 995 1000 1005 1010 1015 1020 1025 1030 1035 1040 1045 1050 1055 1060 1065 1070 1075 1080 1085 1090 1095 1100 1105 1110 1115 1120 1125 1130 1135 1140 1145 1150 1155 1160 1165 1170 1175 1180 1185 1190 1195 1200 1205 1210 1215 1220 1225 1230 1235 1240 1245 1250 1255 1260 1265 1270 1275 1280 1285 1290 1295 1300 1305 1310 1315 1320 1325 1330 1335 1340 1345 1350 1355 1360 1365 1370 1375 1380 1385 1390 1395 1400 1405 1410 1415 1420 1425 1430 1435 1440 1445 1450 1455 1460 1465 1470 1475 1480 1485 1490 1495 1500 1505 1510 1515 1520 1525 1530 1535 1540 1545 1550 1555 1560 1565 1570 1575 1580 1585 1590 1595 1600 1605 1610 1615 1620 1625 1630 1635 1640 1645 1650 1655 1660 1665 1670 1675 1680 1685 1690 1695 1700 1705 1710 1715 1720 1725 1730 1735 1740 1745 1750 1755 1760 1765 1770 1775 1780 1785 1790 1795 1800 1805 1810 1815 1820 1825 1830 1835 1840 1845 1850 1855 1860 1865 1870 1875 1880 1885 1890 1895 1900 1905 1910 1915 1920 1925 1930 1935 1940 1945 1950 1955 1960 1965 1970 1975 1980 1985 1990 1995 2000 2005 2010 2015 2020 2025 2030 2035 2040 2045 2050 2055 2060 2065 2070 2075 2080 2085 2090 2095 2100 2105 2110 2115 2120 2125 2130 2135 2140 2145 2150 2155 2160 2165 2170 2175 2180 2185 2190 2195 2200 2205 2210 2215 2220 2225 2230 2235 2240 2245 2250 2255 2260 2265 2270 2275 2280 2285 2290 2295 2300 2305 2310 2315 2320 2325 2330 2335 2340 2345 2350 2355 2360 2365 2370 2375 2380 2385 2390 2395 2400 2405 2410 2415 2420 2425 2430 2435 2440 2445 2450 2455 2460 2465 2470 2475 2480 2485 2490 2495 2500 2505 2510 2515 2520 2525 2530 2535 2540 2545 2550 2555 2560 2565 2570 2575 2580 2585 2590 2595 2600 2605 2610 2615 2620 2625 2630 2635 2640 2645 2650 2655 2660 2665 2670 2675 2680 2685 2690 2695 2700 2705 2710 2715 2720 2725 2730 2735 2740 2745 2750 2755 2760 2765 2770 2775 2780 2785 2790 2795 2800 2805 2810 2815 2820 2825 2830 2835 2840 2845 2850 2855 2860 2865 2870 2875 2880 2885 2890 2895 2900 2905 2910 2915 2920 2925 2930 2935 2940 2945 2950 2955 2960 2965 2970 2975 2980 2985 2990 2995 3000 3005 3010 3015 3020 3025 3030 3035 3040 3045 3050 3055 3060 3065 3070 3075 3080 3085 3090 3095 3100 3105 3110 3115 3120 3125 3130 3135 3140 3145 3150 3155 3160 3165 3170 3175 3180 3185 3190 3195 3200 3205 3210 3215 3220 3225 3230 3235 3240 3245 3250 3255 3260 3265 3270 3275 3280 3285 3290 3295 3300 3305 3310 3315 3320 3325 3330 3335 3340 3345 3350 3355 3360 3365 3370 3375 3380 3385 3390 3395 3400 3405 3410 3415 3420 3425 3430 3435 3440 3445 3450 3455 3460 3465 3470 3475 3480 3485 3490 3495 3500 3505 3510 3515 3520 3525 3530 3535 3540 3545 3550 3555 3560 3565 3570 3575 3580 3585 3590 3595 3600 3605 3610 3615 3620 3625 3630 3635 3640 3645 3650 3655 3660 3665 3670 3675 3680 3685 3690 3695 3700 3705 3710 3715 3720 3725 3730 3735 3740 3745 3750 3755 3760 3765 3770 3775 3780 3785 3790 3795 3800 3805 3810 3815 3820 3825 3830 3835 3840 3845 3850 3855 3860 3865 3870 3875 3880 3885 3890 3895 3900 3905 3910 3915 3920 3925 3930 3935 3940 3945 3950 3955 3960 3965 3970 3975 3980 3985 3990 3995 4000 4005 4010 4015 4020 4025 4030 4035 4040 4045 4050 4055 4060 4065 4070 4075 4080 4085 4090 4095 4100 4105 4110 4115 4120 4125 4130 4135 4140 4145 4150 4155 4160 4165 4170 4175 4180 4185 4190 4195 4200 4205 4210 4215 4220 4225 4230 4235 4240 4245 4250 4255 4260 4265 4270 4275 4280 4285 4290 4295 4300 4305 4310 4315 4320 4325 4330 4335 4340 4345 4350 4355 4360 4365 4370 4375 4380 4385 4390 4395 4400 4405 4410 4415 4420 4425 4430 4435 4440 4445 4450 4455 4460 4465 4470 4475 4480 4485 4490 4495 4500 4505 4510 4515 4520 4525 4530 4535 4540 4545 4550 4555 4560 4565 4570 4575 4580 4585 4590 4595 4600 4605 4610 4615 4620 4625 4630 4635 4640 4645 4650 4655 4660 4665 4670 4675 4680 4685 4690 4695 4700 4705 4710 4715 4720 4725 4730 4735 4740 4745 4750 4755 4760 4765 4770 4775 4780 4785 4790 4795 4800 4805 4810 4815 4820 4825 4830 4835 4840 4845 4850 4855 4860 4865 4870 4875 4880 4885 4890 4895 4900 4905 4910 4915 4920 4925 4930 4935 4940 4945 4950 4955 4960 4965 4970 4975 4980 4985 4990 4995 5000 5005 5010 5015 5020 5025 5030 5035 5040 5045 5050 5055 5060 5065 5070 5075 5080 5085 5090 5095 5100 5105 5110 5115 5120 5125 5130 5135 5140 5145 5150 5155 5160 5165 5170 5175 5180 5185 5190 5195 5200 5205 5210 5215 5220 5225 5230 5235 5240 5245 5250 5255 5260 5265 5270 5275 5280 5285 5290 5295 5300 5305 5310 5315 5320 5325 5330 5335 5340 5345 5350 5355 5360 5365 5370 5375 5380 5385 5390 5395 5400 5405 5410 5415 5420 5425 5430 5435 5440 5445 5450 5455 5460 5465 5470 5475 5480 5485 5490 5495 5500 5505 5510 5515 5520 5525 5530 5535 5540 5545 5550 5555 5560 5565 5570 5575 5580 5585 5590 5595 5600 5605 5610 5615 5620 5625 5630 5635 5640 5645 5650 5655 5660 5665 5670 5675 5680 5685 5690 5695 5700 5705 5710 5715 5720 5725 5730 5735 5740 5745 5750 5755 5760 5765 5770 5775 5780 5785 5790 5795 5800 5805 5810 5815 5820 5825 5830 5835 5840 5845 5850 5855 5860 5865 5870 5875 5880 5885 5890 5895 5900 5905 5910 5915 5920 5925 5930 5935 5940 5945 5950 5955 5960 5965 5970 5975 5980 5985 5990 5995 6000 6005 6010 6015 6020 6025 6030 6035 6040 6045 6050 6055 6060 6065 6070 6075 6080 6085 6090 6095 6100 6105 6110 6115 6120 6125 6130 6135 6140 6145 6150 6155 6160 6165 6170 6175 6180 6185 6190 6195 6200 6205 6210 6215 6220 6225 6230 6235 6240 6245 6250 6255 6260 6265 6270 6275 6280 6285 6290 6295 6300 6305 6310 6315 6320 6325 6330 6335 6340 6345 6350 6355 6360 6365 6370 6375 6380 6385 6390 6395 6400 6405 6410 6415 6420 6425 6430 6435 6440 6445 6450 6455 6460 6465 6470 6475 6480 6485 6490 6495 6500 6505 6510 6515 6520 6525 6530 6535 6540 6545 6550 6555 6560 6565 6570 6575 6580 6585 6590 6595 6600 6605 6610 6615 6620 6625 6630 6635 6640 6645 6650 6655 6660 6665 6670 6675 6680 6685 6690 6695 6700 6705 6710 6715 6720 6725 6730 6735 6740 6745 6750 6755 6760 6765 6770 6775 6780 6785 6790 6795 6800 6805 6810 6815 6820 6825 6830 6835 6840 6845 6850 6855 6860 6865 6870 6875 6880 6885 6890 6895 6900 6905 6910 6915 6920 6925 6930 6935 6940 6945 6950 6955 6960 6965 6970 6975 6980 6985 6990 6995 7000 7005 7010 7015 7020 7025 7030 7035 7040 7045 7050 7055 7060 7065 7070 7075 7080 7085 7090 7095 7100 7105 7110 7115 7120 7125 7130 7135 7140 7145 7150 7155 7160 7165 7170 7175 7180 7185 7190 7195 7200 7205 7210 7215 7220 7225 7230 7235 7240 7245 7250 7255 7260 7265 7270 7275 7280 7285 7290 7295 7300 7305 7310 7315 7320 7325 7330 7335 7340 7345 7350 7355 7360 7365 7370 7375 7380 7385 7390 7395 7400 7405 7410 7415 7420 7425 7430 7435 7440 7445 7450 7455 7460 7465 7470 7475 7480 7485 7490 7495 7500 7505 7510 7515 7520 7525 7530 7535 7540 7545 7550 7555 7560 7565 7570 7575 7580 7585 7590 7595 7600 7605 7610 7615 7620 7625 7630 7635 7640 7645 7650 7655 7660 7665 7670 7675 7680 7685 7690 7695 7700 7705 7710 7715 7720 7725 7730 7735 7740 7745 7750 7755 7760 7765 7770 7775 7780 7785 7790 7795 7800 7805 7810 7815 7820 7825 7830 7835 7840 7845 7850 7855 7860 7865 7870 7875 7880 7885 7890 7895 7900 7905 7910 7915 7920 7925 7930 7935 7940 7945 7950 7955 7960 7965 7970 7975 7980 7985 7990 7995 8000 8005 8010 8015 8020 8025 8030 8035 8040 8045 8050 8055 8060 8065 8070 8075 8080 8085 8090 8095 8100 8105 8110 8115 8120 8125 8130 8135 8140 8145 8150 8155 8160 8165 8170 8175 8180 8185 8190 8195 8200 8205 8210 8215 8220 8225 8230 8235 8240 8245 8250 8255 8260 8265 8270 8275 8280 8285 8290 8295 8300 8305 8310 8315 8320 8325 8330 8335 8340 8345 8350 8355 8360 8365 8370 8375 8380 8385 8390 8395 8400 8405 8410 8415 8420 8425 8430 8435 8440 8445 8450 8455 8460 8465 8470 8475 8480 8485 8490 8495 8500 8505 8510 8515 8520 8525 8530 8535 8540 8545 8550 8555 8560 8565 8570 8575 8580 8585 8590 8595 8600 8605 8610 8615 8620 8625 8630 8635 8640 8645 8650 8655 8660 8665 8670 8675 8680 8685 8690 8695 8700 8705 8710 8715 8720 8725 8730 8735 8740 8745 8750 8755 8760 8765 8770 8775 8780 8785 8790 8795 8800 8805 8810 8815 8820 8825 8830 8835 8840 8845 8850 8855 8860 8865 8870 8875 8880 8885 8890 8895 8900 8905 8910 8915 8920 8925 8930 8935 8940 8945 8950 8955 8960 8965 8970 8975 8980 8985 8990 8995 9000 9005 9010 9015 9020 9025 9030 9035 9040 9045 9050 9055 9060 9065 9070 9075 9080 9085 9090 9095 9100 9105 9110 9115 9120 9125 9130 9135 9140 9145 9150 9155 9160 9165 9170 9175 9180 9185 9190 9195 9200 9205 9210 9215 9220 9225 9230 9235 9240 9245 9250 9255 9260 9265 9270 9275 9280 9285 9290 9295 9300 9305 9310 9315 9320 9325 9330 9335 9340 9345 9350 9355 9360 9365 9370 9375 9380 9385 939

as the wick. The wick was placed perpendicular to the bottom of a glass bottle with the wick clip. 200 g of paraffin wax having a melting point of 61°C. was warmed, and then placed in a glass container to produce a candle having a height of 6.5 cm. The candle was allowed to stand at 25°C. 5 for 24 hours to produce a fully hardened candle.

## TEST EXAMPLE 1

The candles produced in Examples 1 to 11 and Comparative Examples 1 to 3 were combusted for 5 hours to evaluate a change in wick over time.

○: The wick was combusted down together with the flame.

Δ: The wick was combusted in a state in which a length of the wick was extended 3 to 5 mm from the top of wax.

×: The wick was combusted in a state in which a length of the wick was extended 5 mm or longer from the top of wax.

TABLE 1

|                       | Change in wick |      |      |      |      |
|-----------------------|----------------|------|------|------|------|
|                       | 1 hr           | 2 hr | 3 hr | 4 hr | 5 hr |
| Example 1             | ○              | ○    | ○    | Δ    | Δ    |
| Example 2             | ○              | ○    | ○    | ○    | Δ    |
| Example 3             | ○              | ○    | ○    | ○    | ○    |
| Example 4             | ○              | ○    | ○    | Δ    | Δ    |
| Example 5             | ○              | ○    | ○    | Δ    | Δ    |
| Example 6             | ○              | ○    | Δ    | Δ    | Δ    |
| Example 7             | ○              | ○    | Δ    | Δ    | Δ    |
| Example 8             | ○              | ○    | Δ    | Δ    | Δ    |
| Example 9             | ○              | ○    | ○    | Δ    | Δ    |
| Example 10            | ○              | ○    | ○    | Δ    | Δ    |
| Example 11            | ○              | ○    | —    | —    | —    |
| Comparative Example 1 | Δ              | Δ    | ×    | ×    | ×    |
| Comparative Example 2 | ○              | Δ    | ×    | ×    | ×    |
| Comparative Example 3 | ○              | Δ    | ×    | ×    | ×    |

Table 1 shows evaluation results of the change in the wick for a candle of over time for each sample. According to Table 1, it could be confirmed that in Examples 1 to 10, the wick was combusted together with flame or the length of the wick was slightly longer over time. In Example 11, it was confirmed that the wick was combusted together with the flame, but the combustion was not possible after 2 hours or longer since the tunnel phenomenon occurred.

In Comparative Example 1, the commercially available cotton wick was used, and it was confirmed that the length of the wick combusted over time was excessively long, i.e., 5 mm or more. In Comparative Example 2, the commercially available smokeless wick was used, and it was confirmed that the combusted wick remained long over time. In Comparative Example 3, the wood wick was used, and it was confirmed that the combusted wick remained long over time.

An image of the sheet produced in Example 1 is shown in FIG. 14. As shown in FIG. 14, pulp and carbon material short fibers formed a matrix. The porosity was measured according to ASTM D-6226 method. It was found that the porosity was 62%, and thus, a number of fine pores were included, as measured using a porosity measuring apparatus (ULTRAFOAM 1200e of Quantachrome Instruments). Further, images of the candles including the wicks produced by cutting the manufactured sheet were shown in FIGS. 15 to 16. FIG. 15 is a front view of the candle, and FIG. 16 is a side view of the candle.

## TEST EXAMPLE 2

The candle samples produced in Examples 1 to 11 and Comparative Examples 1 to 3 were combusted for 5 hours to evaluate occurrence of soot and ash over time.

○: Soot and ash rarely occurred.

Δ: A small amount of soot or ash occurred.

×: A large amount of soot and ash occurred.

TABLE 2

|                       | Occurrence of soot and ash |      |      |      |      |
|-----------------------|----------------------------|------|------|------|------|
|                       | 1 hr                       | 2 hr | 3 hr | 4 hr | 5 hr |
| Example 1             | ○                          | ○    | ○    | ○    | Δ    |
| Example 2             | ○                          | ○    | ○    | ○    | Δ    |
| Example 3             | ○                          | ○    | ○    | ○    | ○    |
| Example 4             | ○                          | ○    | ○    | ○    | Δ    |
| Example 5             | ○                          | ○    | ○    | Δ    | Δ    |
| Example 6             | ○                          | ○    | Δ    | Δ    | Δ    |
| Example 7             | ○                          | ○    | Δ    | Δ    | Δ    |
| Example 8             | ○                          | ○    | Δ    | Δ    | Δ    |
| Example 9             | ○                          | ○    | ○    | Δ    | Δ    |
| Example 10            | ○                          | ○    | ○    | Δ    | Δ    |
| Example 11            | ○                          | ○    | —    | —    | —    |
| Comparative Example 1 | Δ                          | ×    | ×    | ×    | x    |
| Comparative Example 2 | ○                          | Δ    | ×    | ×    | x    |
| Comparative Example 3 | ○                          | Δ    | ×    | ×    | x    |

Table 2 shows evaluation results of occurrence of soot and ash for each sample. As shown in Table 2, it was confirmed that in the wicks of Examples 1 to 5 and Examples 9 and 10, little or only a small amount of smoke, soot and ash occurred at the time of combustion for 3 hours or more. It could be confirmed that in the wicks of Examples 6 to 8, some smoke occurred at the time of combustion for 2 hours or longer, but 35 soot and ash did not remain black. In the wick of Example 11, soot and ash did not occur at the time of combustion for 2 hours or longer, but the combustion was not possible after 2 hours or longer due to the tunnel phenomenon.

In the wicks of Comparative Examples 1 to 3, it could be 40 confirmed that soot and ash did not occur in a large amount at an initial stage, but soot and ash excessively occurred over time at the time of combustion for 1 hour or more. It could be confirmed that in the wood wick of Comparative Example 3, black smoke occurred at the time of combustion, 45 and soot also occurred very seriously over time.

Since the wick for the candle according to the present invention includes the carbon material, the length of the wick is not longer than that of the conventional wick after combustion, and thus, it is convenient to use the wick for the candle since it is not required to cut the wick separately.

Further, the phenomenon in which the ash of the wick falls due to combustion is remarkably reduced, and thus, the candle is not stained, and it is clearly combusted in view of aesthetic aspect.

55 In addition, occurrence of smoke and soot due to combustion may be remarkably reduced.

Further, the tunnel phenomenon due to the thermal conduction of the wick may be suppressed.

As described above, although preferred embodiments of 60 the present invention are described, the present invention should be construed as including all the changes, modification, and equivalent, such that it is obvious that the present invention may be equivalently utilized by appropriately modifying the above-described exemplary embodiments. Therefore, the above-description is not intended to limit the 65 scope of the present invention defined by limitation of the following claims.

19

What is claimed is:

1. A wick for a candle comprising a carbon material vaporized into carbon dioxide gas at a time of combustion, wherein the carbon material is any one or a mixture or a composite of two or more selected from carbon fiber, activated carbon, carbon nanotube, graphite, carbon black, graphene, graphene oxide, and a carbon composite material, and the carbon material is dispersed in a matrix forming the wick.
2. The wick for a candle of claim 1, wherein the carbon material has a form of any one or two or more selected from long fibers, short fibers, fabrics and particles.
3. The wick for a candle of claim 2, wherein the wick is selected from the following (i) to (v):
  - (i) a wick formed of the carbon material alone,
  - (ii) a wick in which the carbon material is dispersed in a matrix formed of any one selected from a binder and pulp, or a mixture thereof,
  - (iii) a wick including the carbon material in a fabric formed of any one or two or more fibers selected from natural fibers and synthetic fibers,
  - (iv) a wick including the carbon material in the fabric formed of any one or two or more fibers selected from natural fibers and synthetic fibers, the fabric being coated or impregnated with a binder, and
  - (v) a wick including the carbon material and any one or two or more short fibers selected from short fibers of natural fibers and short fibers of synthetic fibers, in the matrix formed of any one selected from a binder and pulp, or a mixture thereof.

20

4. The wick for a candle of claim 3, wherein the wick has a web form including pores in the wick to allow fuel of the candle to be moved by a capillary phenomenon.

5. The wick for a candle of claim 3, further comprising: a supporter selected from a wood wick, a zinc wick, a tin wick, and a zinc-tin mixed metal wick.

6. The wick for a candle of claim 3, wherein the binder has a melting temperature satisfying Equation 1 below:

$$\text{melting temperature of fuel used in candle} < \text{melting temperature of binder.} \quad [\text{Equation 1}]$$

7. The wick for a candle of claim 1, wherein the wick is coated with wax.

8. The wick for a candle of claim 1, further comprising: a wick clip.

9. A candle comprising the wick for a candle of claim 1.

10. The candle of claim 9, wherein the candle includes any one or two or more fuels selected from paraffin wax, paraffin oil, soy wax, bees wax, palm wax, and gel wax.

11. The candle of claim 10, wherein the fuel further includes any one or two or more additives selected from fragrance and dye.

12. The wick of a candle of claim 3, wherein the wick is formed of a sheet including carbon material short fibers, pulp and a binder, in which the pulp is fibrillated cellulose-based fiber having a three-dimensional mesh structure, and the carbon material short fibers are dispersed in the wick.

\* \* \* \* \*